

## UNITED STATES PATENT OFFICE

2,202,641

## EXTREME PRESSURE LUBRICANT

Darwin E. Badertscher and Henry G. Berger,  
Woodbury, and Francis M. Seger, Pitman, N. J.,  
assignors to Socony-Vacuum Oil Company, In-  
corporated, New York, N. Y., a corporation of  
New York

No Drawing. Application November 23, 1937,  
Serial No. 176,054

7 Claims. (Cl. 87—9)

This invention has to do in a general way with lubricating materials and is more particularly related to improved lubricating compositions adapted for use under abnormally high pressure conditions.

It is well known to those familiar with the art that a lubricating oil such as a mere refined petroleum oil fraction is incapable of maintaining a lubricating film between engaged metallic surfaces where the unit load at the engaged surfaces exceeds a pressure of say 3000—4000 lbs. per square inch. In various types of modern machinery, such as the hypoid gears used in motor vehicles, the engaging pressures between the gear teeth are so high that they are incapable of proper lubrication by the so-called "thick film" which is obtained through the use of oils of the type above referred to. It has, therefore, become the practice to incorporate in lubricating oils of this type an additive ingredient which will form, or which is capable of reaction under extreme pressure conditions to form, a lubricant film capable of withstanding these high pressures. Ingredients of this character are known as extreme pressure ingredients or extreme pressure (E. P.) lubricant bases and the lubricant compositions compounded with a minor proportion of such ingredients are known as E. P. lubricants.

Numerous materials have been proposed for use as E. P. bases and among such materials have been proposed compounds or materials containing sulfur and chlorine. The present invention is related to this latter type or class of materials. It is the primary object of this invention to provide an extreme pressure lubricant compounded with a chlorine and sulfur containing E. P. base which may be easily and economically manufactured and which is stable within the oil under conditions of storage and use.

More specifically our invention is based upon the discovery that a highly efficient extreme pressure lubricant base can be formed as the reaction product of a halogenated organic compound, preferably aliphatic, with an alkali thiocyanate.

The particular compounds representative of the class contemplated by this invention are obtained by reacting an alkali thiocyanate with a chlorinated petroleum naphtha, the proportions of the reactants being such that the final product contains both chlorine and sulfur.

Chlorinated petroleum naphtha or chlornaphtha can be prepared by chlorinating a petroleum naphtha such as Stoddard Solvent to a chlorine content of from about 25% to about 50%. Chlorinated naphtha obtained in this way can then be re-

acted with an alkali thiocyanate to effect a replacement of part of the chlorine with the thiocyanate group. The proportions of chlorine and sulfur in the final product may be varied by varying the chlorination of the chlornaphtha and also by varying the proportions of the chlorinated aliphatic compound (chlornaphtha) and the alkali thiocyanate in the final reaction. Compounds formed in this way are, for the purpose of description and definition herein, referred to specifically as chlornaphtha thiocyanates and broadly as halogenated aliphatic thiocyanates.

To illustrate the manner in which halogen (chlorine)-substituted aliphatic compounds of the type contemplated by this invention may be formed, we have described, in the following two examples, procedures which may be followed in the syntheses of chlornaphtha thiocyanates.

*Example 1.*—A mixture of 50 grams of potassium thiocyanate, 170 grams of chlorinated naphtha containing 51.8% chlorine, and 200 cc. of acetone was heated and stirred at a temperature of from 40° C. to 50° C. over a period of two hours. The mixture was filtered free of solid materials and the solvent distilled off. The residue thus obtained was again filtered, yielding an oil-miscible product containing 43.66% chlorine and 1.6% sulfur.

*Example 2.*—A mixture of 50 grams of potassium thiocyanate, 100 grams of chlorinated naphtha containing 48.3% chlorine, and 200 cc. of acetone was stirred and refluxed over two hours. The resulting mixture was subjected to the same refining operation described in Example 1 and yielded an oil-miscible liquid product containing 41% chlorine and 2.8% sulfur.

To demonstrate the value of chlorine-thiocyanate substituted aliphatic compounds of the type contemplated by this invention as extreme pressure lubricant bases, we have prepared lubricant compositions using the chlornaphtha thiocyanates obtained from the two examples above, in a mineral oil having a S. U. viscosity of 80—90 seconds at 210° F. These extreme pressure lubricant compositions have been subjected to the Almen Pin Test (Wolf and Mougey, Proc. A. P. I. 1932, pp. 118—130) and the S. A. E. Test (S. A. E. Journal 39, 23—4 (1936)). These tests are commonly accepted as standard for determining extreme pressure lubricant characteristics of lubricant compositions and in the table below we have shown the results obtained with these tests, using the unblended or untreated oil above referred to and samples of the same oil blended with a minor proportion of the two chlornaphtha

thiocyanate compositions obtained in Examples 1 and 2 given above. The additive ingredient in each case is identified by the example number used above, and the table, it will be observed, 5 shows that these compounds were added to the oil in concentrations of 5% and 10%.

*E. P. tests (pounds failed)*

| 10 | Product                          | Per-<br>cent<br>in oil | Almen              | S. A. E./R. P. M.<br>rubbing ratio<br>14.6:1 loading<br>rate 63.5 lbs./sec. |
|----|----------------------------------|------------------------|--------------------|-----------------------------------------------------------------------------|
| 15 | Untreated oil.....               |                        | 3000-4000          | R. P. M.<br>40-70/755<br>10-15/1000                                         |
|    | Material from Example No. 1..... | 10<br>5                | 30,000+<br>30,000+ | 580+/-755<br>430/1000                                                       |
|    | Material from Example No. 2..... | 10<br>5                | 30,000+<br>30,000+ | 340/1000<br>300/1000                                                        |

20 It will be seen from the foregoing table that the chlorine-thiocyanate substituted aliphatic hydrocarbons contemplated by this invention, when blended with a mineral oil in minor proportions, are effective to greatly improve the load carrying 25 capacity of such oil and it is to be understood that while we have illustrated our invention with certain specific examples, using a particular halogenated aliphatic compound (chlornaphtha) and a particular alkali thiocyanate (potassium thiocyanate) and have described certain exemplary 30 procedures for preparing the compounds, the invention is not limited to the specific examples either as to ingredients or procedure. It is also to be understood that while we have illustrated 35 our extreme pressure lubricant composition as comprising a mineral lubricating oil as the preferred carrier for the E. P. base or ingredient, our invention is not necessarily restricted to extreme pressure lubricants compounded with mineral oil as the carrying agent but contemplates other suitable carrying mediums, such as lighter petroleum fractions, fatty vegetable or animal oils, benzene and similar hydrocarbons, alcohols, ethers, esters, and media in which our E. P. base 40 may be dissolved, dispersed, or emulsified.

We claim:

1. An extreme pressure lubricant comprising a

hydrocarbon lubricant oil and in admixture therewith a minor proportion of the oil-miscible product obtained by the reaction of a halogenated aliphatic hydrocarbon and an alkali thiocyanate in such proportions that said product contains both sulfur and chlorine.

2. An extreme pressure lubricant comprising a hydrocarbon lubricant oil and in admixture therewith a minor proportion, from about 0.5% to 10%, of the oil-miscible product obtained by 10 the reaction of a chlorinated aliphatic hydrocarbon and an alkali thiocyanate in such proportions that said product contains both sulfur and chlorine.

3. An extreme pressure lubricant comprising a hydrocarbon lubricant oil and in admixture therewith a minor proportion of the oil-miscible product obtained by the reaction of a chlorinated aliphatic hydrocarbon and an alkali thiocyanate in such proportions that said product contains 20 both sulfur and halogen.

4. An extreme pressure lubricant comprising a hydrocarbon lubricant oil and in admixture therewith a minor proportion of a chlorine and thiocyanate substituted aliphatic hydrocarbon. 25

5. An extreme pressure lubricant comprising a hydrocarbon lubricant oil and in admixture therewith a minor proportion of chlornaphtha thiocyanate obtained by reacting a chlorinated petroleum naphtha with an alkali thiocyanate in 30 such proportions that the reaction product contains a residual amount of chlorine.

6. An extreme pressure lubricant comprising a hydrocarbon lubricant oil and in admixture therewith a minor proportion, from about 0.5% 35 to about 10%, of chlornaphtha thiocyanate obtained by reacting a chlorinated petroleum naphtha with an alkali thiocyanate in such proportions that the reaction product contains a residual amount of chlorine.

7. An extreme pressure lubricant comprising a hydrocarbon lubricating oil and in admixture therewith a minor proportion of a halogenated aliphatic thiocyanate.

DARWIN E. BADERTSCHER. 45  
HENRY G. BERGER.  
FRANCIS M. SEGER.